# EUROPEAN PATENT SPECIFICATION

(11) **EP 0 302 676 B1**
(45) Date of publication and mention of the grant of the patent: **17.07.1991**
(21) Application number: 88307050.0
(22) Date of filing: 29.07.1988
(51) Int. Cl.: F04C 18/34, F01C 21/08

(54) **Rotor vanes**
Flügel für Rotoren
Palettes pour rotor

(30) Priority: 03.08.1987 GB 8718312
(43) Date of publication of application: 08.02.1989
(73) Proprietor: ROTOCOLD HOLDINGS LIMITED, Bradford, West Yorkshire BD1 5BS (GB)
(72) Inventor: Wood, Richard, Canon Pyon Hereford (GB)
(74) Representative: Shaw, Laurence

(56) References cited:
- EP-A- 0 019 605
- GB-A- 1 324 443
- GB-A- 1 336 128
- US-A- 4 209 286

## Description

The invention relates to a rotor compressor of the type having movable vanes located in sockets in the rotor, the rotor being housed in a chamber having an inlet port for refrigerant gas to be drawn into the chamber and an outlet port spaced from the inlet port for discharge of the gas, the vanes defining between the inlet and the outlet at least one suction cell and at least one compression cell. Such compressors are exemplified by the disclosure of US patent 4049410.

It also relates to a vane for such a compressor and a method of manufacturing such a vane.

It is known to make the vanes by injection moulding a composition comprising a polymer, a reinforcing carbon fibre and a lubricant.

EP-A-0019605 discloses a rotary machine having vanes comprising a matrix of a fluorocarbon polymer, e.g. polytetrafluoroethylene, and from 5 to 30% by volume of an inorganic solid lubricant and lirewise 5-30% by volume of carbon fibres. GB-A-1336128 discloses rotor blades for rotary compressors and vacuum pumps comprising a plastics material containing 5 to 33 1/3% of carbon fibre, based an the total weight of fibrous components, said fibrous components constituting 30% to 70% of the total weight of the plastics material. The fibres may be randomly oriented.

It has now been discovered that if the content of the carbon fibre and of the polytetrafluoroethylene used as lubricant are in defined limits, certain benefits result.

According to one aspect of the invention there is provided a rotary compressor comprising a housing including a chamber housing a rotor having rotor vanes, an inlet port and an outlet port being present in the wall of the chamber, the rotor vanes being located in sockets radially spaced about the rotor, the vanes being movable in their sockets and having been injection moulded of a composition comprising a mouldable plastics, from 5 to 30% by volume of a lubricant and 5 to 30% by volume of reinforcing carbon fibres characterised in that the lubricant is polytetrafluroethylene and makes up 5 to 12% by weight of the composition and the reinforcing carbon fibres are randomly oriented and make up 22 to 32% by weight of the composition.

Our evaluations have shown that to achieve a satisfactory combination of ease of moulding of the composition in manufacture and performance of the vanes in service, it is necessary to proportion the quantity of carbon fibre content in the specified range. Particular factors to be considered in service, especially at the tip of the blade, are wear, susceptibility to friction and degradation. Strength, mechanical stability and weight are also important, especially for the body of the blade.

Cost is also a factor. By controlling the content of carbon fibre and also of the lubricant (as indicated below), the desired properties are achieved. More specifically, if the content of carbon fibre falls below the minimum level specified, the blade strength is reduced below an acceptable level. If the content exceeds the upper limit, the wear rate on the rotor and compressor profile increases to unacceptable levels. If the carbon fibre content is kept within the limits specified, the vanes have a long wear resistant life without breakage.

If the polytetrafluoroethylene content exceeds the upper limit, then the lubricant promotes excessive creep of the blade material on the high pressure reaction surfaces of the blades such as the trailing edge in proximity to the corner of the rotor slot and leads to premature failure.

The invention includes rotor vanes per se. The vanes may take any known shape and will usually have a rectangular body and may include grooves on one side.

## Claims

1. A rotary compressor comprising a housing including a chamber housing a rotor having rotor vanes, an inlet port and an outlet port being present in the wall of the chamber, the rotor vanes being located in sockets spaced about the rotor, the vanes being movable in their sockets and having been injected moulded of a composition comprising a mouldable plastics, from 5 to 30% by volume of a lubricant and 5 to 30% by volume of reinforcing carbon fibres characterised in that the lubricant is polytetrafluoroethylene and makes up 5 to 12% by weight of the composition and the reinforcing carbon fibres are randomly oriented and make up 22 to 32% by weight of the composition.

2. A rotor blade comprising a rectangular body adapted to be received at least in part in a socket therefor in a rotor, the blade having been moulded of a composition comprising a mouldable plastics, from 5 to 30% by volume of a lubricant and 5 to 30% by volume of reinforcing carbon fibres characterised in that the lubricant is polytetrafluoroethylene and makes up 5 to 12% by weight of the composition and the reinforcing carbon fibres are randomly oriented and make up 22 to 32% by weight of the composition.

3. A method of making a rotor blade to be received at least in part in a socket therefor in a rotor, the method comprising injection moulding the blade of a composition comprising a mouldable plastics, from 5 to 30% by volume of a lubricant and from 5 to 30% by volume of reinforcing carbon fibres characterised in that the lubricant is polytetrafluoroethylene and makes up 5 to 12% by weight of the composition and the reinforcing carbon fibres are randomly oriented and make up 22 to 32% by weight of the composition.

## Patentansprüche

1. Ein Rotationskompressor umfassend ein Gehäuse mit einer Kammer, die einen Rotor mit Rotorblällern Aufnimmt, wobei die Wand der Kammer eine Einlaßöffnung und eine Auslaßöffnung aufweist, wobei sich die Rotorblätter in Halterungen befinden, die um den Rotor herum angeordnet sind, wobei die Rotoren in ihren Halterungen beweglich sind und aus einem Gemisch aus formbarem Kunststoff aus 5 bis 30 Vol.-% eines Schmiermittels und 5 bis 30 Vol.-% Verstärkungskohlenstoffasern spritzgegossen wurden, dadurch gekennzeichnet, daß das Schmiermittel Polytetrafluorethylen ist und 5 bis 12 Gew.-% des Gemisches ausmacht und die Verstärkungskohlenstoffasern zufallsorientiert sind und 22 bis 32 Gew.-% des Gemisches ausmachen.

2. Ein Rotorblatt mit einem rechteckigen Körper, der wenigstens telweise in einer in einem Rotor hierfür vorgesehenen Halterung aufgenommen wird, wobei das Blatt aus einem Gemisch aus einem formbaren Kunststoff aus 5 bis 30 Vol.-% eines Schmiermittels und 5 bis 30 Vol.-% Verstärkungskohlenstoffasern gegossen wurde, dadurch gekennzeichnet, daß das Schmiermittel Polytetrafluorethylen ist und 5 bis 12 Gew.-% des Gemisches ausmacht und 22 bis 32 Gew.-% des Gemisches ausmachen.

3. Verfahren zur Herstellung eines Rotorblattes, das wenigstens teilweise in einer in einem Rotor hierfür vorgesehenen Halterung aufgenommen wird, umfassend die folgenden Schritte: Spritzgießen des Blattes mit einem Gemisch aus 5 bis 30 Vol.-% eines Schmiermittels und 5 bis 30 Vol.-% Verstärkungskohlenstoffasern, dadurch gekennzeichnet, daß das Schmiermittel Polytetrafluorethylen ist und 5 bis 12 Gew.-% des Gemisches ausmacht und die Verstärkungskohlenstoffasern zufallsorientiert sind und 22 bis 32 Gew.-% des Gemisches ausmachen.

## Revendications

1. Compresseur rotatif comprenant un châssis qui inclut une chambre renfermant un rotor muni de pales, avec un orifice d'entrée et un orifice de sortie dans la paroi de la chambre, les pales du rotor étant situées dans des cavités autour du rotor, les pales pouvant se déplacer dans leurs cavités et ayant été moulées par injection à partir d'un matériau comprenant des plastiques de moulage, 5 à 30% du volume étant constitué par un lubrifiant et 5 à 30% du volume par des fibres de carbone de renforcement, caractérisé en ce que le lubrifiant est du polytétrafluoroéthylène et que son poids constitue de 5 à 12% du poids du matériau, et que les fibres de carbone de renforcement sont orientées au hasard et constituent de 22 à 32% du poids du matériau.

2. Lame de rotor comprenant un corps rectangulaire adapté pour être fixé au moins en partie dans la cavité d'un rotor comme préalablement indiqué, la lame ayant été moulée à partir d'un matériau comprenant des plastiques de moulage, 5 à 30% du volume étant constitué d'un lubrifiant et 5 à 30% du volume de fibres de carbone de renforcement, caractérisée en ce que le lubrifiant est du polytétrafluoroéthylène et que son poids constitue de 5 à 12% du poids du matériau et que les fibres de carbone de renforcement sont orientées au hasard et constituent de 22 à 32% du poids du matériau.

3. Méthode de fabrication d'une pale de rotor à fixer au moins en partie dans la cavité d'un rotor comme préalablement indiqué, la méthode comprenant le moulage par injection d'une lame à partir d'un matériau comprenant des plastiques de moulage, 5 à 30% du volume étant constitué d'un lubrifiant et 5 à 30% du volume de fibres de carbone de renforcement, caractérisée en ce que le lubrifiant est du polytétrafluoroéthylène et constitue de à 12% du poids du matériau et que les fibres de carbone de renforcement sont orientées au hasard et constituent de 22 à 32% du poids du matériau.
